

P. R. HEYL,  
TERMINAL FOR CONTACT OR SPARK DEVICES,  
APPLICATION FILED MAR. 20, 1915.  
1,166,129.

Patented Dec. 28, 1915.



Inventor:  
Paul R. Heyl  
by his Atty's:  
Philip Sawyer & Robert Kennedy

# UNITED STATES PATENT OFFICE.

PAUL R. HEYL, OF NEW ROCHELLE, NEW YORK, ASSIGNOR TO COMMERCIAL RESEARCH COMPANY, OF NEW YORK, N. Y., A CORPORATION OF NEW YORK.

## TERMINAL FOR CONTACT OR SPARK DEVICES.

1,166,129.

Specification of Letters Patent. Patented Dec. 28, 1915.

Application filed March 20, 1915. Serial No. 15,983.

*To all whom it may concern:*

Be it known that I, PAUL R. HEYL, a citizen of the United States, residing at New Rochelle, county of Westchester, and State 5 of New York, have invented certain new and useful Improvements in Terminals for Contact or Spark Devices, fully described and represented in the following specification and the accompanying drawings, forming 10 a part of the same.

This invention relates to improvements in terminals for contact or spark devices.

It has been the usual practice heretofore to provide a contact device or spark point 15 in electrical apparatus with a terminal facing or cap of platinum in order to insure that such facing or cap will remain clean and unaffected by electric sparks which may be formed between such terminal facings.

Platinum has been employed for such terminal facings particularly on account of 20 its high melting point and its nonoxidizability or chemical inertness under various conditions of service, whereby it maintains 25 a good metallic surface even though heated to a relatively high temperature by the sparks. Hardness has generally been considered an advantage in a terminal facing for a contact device where the points are 30 moved into and out of contact with each other. In fact it has sometimes been the practice to alloy a certain percentage of 35 iridium with platinum in order to produce a terminal facing of greater hardness. I have found, however, that in practice it is difficult to make the contact surfaces fit 40 exactly to each other throughout their entire extent, and therefore with very hard terminal facings any defect in accurate fitting of the meeting surfaces becomes a disadvantage, because the surfaces do not thereafter wear to a good contact with each other, or at least not for a long time.

I have found that a terminal facing for 45 spark points or contact devices comprising a mixture of palladium and silver has important advantages over anything heretofore known to me. Palladium is a material having a high melting point, but when alloyed with silver the melting point of the 50 alloy is very considerably reduced. This apparently would be a great disadvantage and would seem to indicate that such an alloy would not be satisfactory for the pur-

poses named. I have found, however, that 55 as the thermal-conductivity of silver is very high, when mixed with palladium it gives to the alloy a thermal-conductivity considerably above that of palladium. Owing to this thermal-conductivity the heat generated 60 by the spark is conducted away from the contact surface rapidly enough to insure that the surface portion will not reach a temperature above the melting point of the alloy. Where the current passing through 65 the terminal facings does not have a great density, the terminal facings may be formed of an alloy composed principally of silver with a relatively small amount of palladium. In fact I have found that an alloy of silver 70 with 2 per cent. of palladium will give satisfactory results under many circumstances. When, however, the spark points or contact devices are to be exposed to an atmosphere containing sulfur compounds, the percentage 75 of palladium should be increased. I have found that an alloy of silver with 5 per cent. of palladium or more is substantially inert in any atmosphere likely to be 80 encountered in practice.

A further important feature of my invention, however, consists in a special proportioning of the constituents of such an alloy, and is not limited to an alloy of palladium and silver. It will be noted that palladium is a nonoxidizable metal having a high melting point but a low thermal-conductivity. Silver on the other hand is a metal having a comparatively low melting point but a high thermal-conductivity. 85 When, in an alloy of palladium and silver, the percentage of palladium is increased, the melting point of the alloy is increased, but its thermal-conductivity is decreased. At a certain intermediate point between the 90 maximum and minimum proportions of palladium, the alloy will have the maximum resistance to spark erosion for an alloy of such components. The particular percentage which produces this maximum above 100 mentioned may be considered as a critical proportion, because if the percentage of palladium be increased the thermal-conductivity of the alloy is decreased, and, hence, for this reason its resistance to spark erosion 105 is reduced, whereas if the percentage of silver is increased from said critical proportion, the melting point of the alloy is de-

creased, and for this reason its resistance to spark erosion is reduced. I have found that such a critical proportion for a palladium-silver alloy occurs with about 60 per cent. of silver and 40 per cent. of palladium. When an alloy of this composition is used for the terminal facings of contact devices or spark points the result will be entirely satisfactory with the greatest density of current encountered in practice, while at the same time such an alloy is substantially mechanically inert and will not be affected by the reacting components of any atmosphere likely to be encountered in practice. It is to be understood that considerable variation from the critical proportion may obtain in practice without material disadvantage. In fact I have found that 50 to 80 per cent. of palladium and 50 to 20 per cent. of silver form an alloy particularly satisfactory for general use. It is clear that so far as this feature of my invention is concerned, any non-oxidizable high melting metal of low thermal-conductivity may be combined with a low melting metal of high thermal-conductivity in substantially the proper critical proportion so as to produce an alloy having the maximum resistance to spark erosion.

In the accompanying drawing, I have illustrated three curves, A, B, and C. Two of these curves, A and B, respectively show the thermal-conductivity and the melting point of alloys of palladium and silver of different proportions. In this diagram the percentages of palladium have been plotted as abscissae, while the ordinates corresponding thereto indicate on curve B the melting points of the respective compositions and on curve A the thermal-conductivities of said compositions. It will be noted that where the percentage of silver is zero, that is to say, where the composition is pure palladium, the melting point is a maximum. Where the percentage of silver is 100, that is to say, where the composition is pure silver, the thermal-conductivity is a maximum.

In view of my discovery that the alloy which has substantially about 60 per cent. of silver and 40 per cent. of palladium has the maximum resistance to spark erosion, the curves A and B may be so plotted that they will cross at the point corresponding to this particular alloy. Since the resistance to spark erosion falls off when the proportions of the alloy are varied either way from the critical proportion, a curve may be drawn to represent this resistance to spark erosion, and it will be found that for practical purposes the first part of the curve of resistance to spark erosion may be assumed to follow the first part of the curve B, while the last part follows the last part of the curve B. Of course, the form and

size of the contact point will affect the conductivity and radiation so that for this and other reasons the curve of resistance to spark erosion may not follow exactly the curve laid down as proposed above, but for purposes of illustration of the present invention, and for practical purposes in preparing other alloys the plan suggested may be followed with satisfactory results. It is to be understood, however, that these curves are merely illustrative and are introduced principally for the purpose of giving an explanation of why a terminal comprising a high melting metal and a metal of high thermal conductivity will give a maximum resistance to spark erosion when combined in a certain critical proportion. Therefore, for the purpose of illustration, from the curves A and B may be deduced a curve C, indicating the resistance to spark erosion of an alloy of different proportions. It will be seen that this curve C reaches a maximum at a point where the alloy comprises about 40% of silver and 60% of palladium. At this critical proportion the melting point of the composition is the highest obtainable in such an alloy simultaneously with the highest thermal-conductivity of such alloy. That is to say, the alloy has the maximum resistance to spark erosion. The same principle is applicable to other alloys comprising nonoxidizable high melting metals of low thermal-conductivity, and relatively low melting metals of high thermal-conductivity.

From curve C it will be noted that for a considerable distance at each side of the maximum the curvature is relatively flat, so that, for example, between the ordinates indicating 40 and 80% respectively of palladium, the resistance to spark erosion does not change greatly. Hence, with this alloy the proportions of palladium may be varied from 40 to 80% without material disadvantage even under conditions where the terminals are subjected to severe conditions of service.

A terminal facing for a contact device made of palladium-silver alloy may be somewhat softer than pure platinum, whereby considerable difficulty in fitting the surfaces to each other is avoided owing to the fact that as the composition is somewhat softer and more malleable than platinum the hammering of the contact surfaces against each other in practice will force an accurate fit of the contact surfaces, and thereby insure a satisfactory operation of the contacts, even when not accurately fitted initially. Of course, the contacts should not be so soft as to materially flatten out after the surfaces have been brought into contact throughout.

In practice I have found that terminal facings comprising an alloy of palladium and silver are as satisfactory as pure plati-

num facings, while at the same time they are more readily worked into shape and attached in place by soldering or the like.

While I have particularly referred to a terminal facing consisting of palladium and silver alloy, it is to be understood that my invention in its broadest aspect does not exclude such an alloy containing other constituents in addition to the palladium and silver.

10 What is claimed is:

1. A terminal for an electric spark or contact device comprising palladium and silver.
2. A terminal for an electric spark or contact device consisting of an alloy of palladium and silver.
3. A terminal for an electric spark or contact device consisting of an alloy of palladium and silver containing from substantially 40 to 80 per cent. of palladium.

20

dium and silver containing from substantially 40 to 80 per cent. of palladium.

4. A terminal for an electric spark or contact device consisting of an alloy comprising a nonoxidizable metal having a high melting point and low thermal-conductivity, and a metal having a low melting point and a high thermal-conductivity, the metals being combined in substantially such proportions as to give the alloy a maximum resistance to spark erosion, substantially as described.

25

In testimony whereof, I have hereunto set my hand, in the presence of two subscribing witnesses.

30 PAUL R. HEYL.

Witnesses:

BENJ. B. RILEY,  
CHAS. D. AYLES.